

L. J. PEARSON AND W. E. HOLLAND,  
STORAGE BATTERY GRID AND METHOD OF MAKING SAME,  
APPLICATION FILED DEC. 9, 1919.

1,384,875.

Patented Mar. 23, 1920.

Fig. 1.



Fig. 2.

Inventors.—

Lawrence J. Pearson,  
Walter E. Holland.

by their Attorneys  
Fowson & Fowson

# UNITED STATES PATENT OFFICE.

LAWRENCE J. PEARSON, OF WILLOW GROVE, AND WALTER E. HOLLAND, OF PHILADELPHIA, PENNSYLVANIA, ASSIGNEES TO PHILADELPHIA STORAGE BATTERY COMPANY, OF PHILADELPHIA, PENNSYLVANIA, A CORPORATION OF PENNSYLVANIA.

## STORAGE-BATTERY GRID AND METHOD OF MAKING SAME.

1,834,875.

Specification of Letters Patent. Patented Mar. 23, 1920.

Continuation of application Serial No. 240,789, filed June 19, 1918. This application filed December 9, 1919. Serial No. 343,521.

To all whom it may concern:

Be it known that we, LAWRENCE J. PEARSON and WALTER E. HOLLAND, citizens of the United States, residing in Willow Grove and Philadelphia, respectively, in the State of Pennsylvania, have invented Storage-Battery Grids and Methods of Making Same, of which the following is a specification.

10 One object of our invention is to provide a storage battery grid which shall not warp nor prematurely disintegrate under conditions of use and which as a consequence shall have an increased useful life;—the invention contemplating more particularly a cast metal grid whose structure shall be of uniform density and character at all points, free from blow holes and close grained so that when embodied in a battery

20 plate it shall be attacked to a minimum and uniform extent by the electrolytic action during charging and discharging of the battery.

These objects and other advantageous ends 25 we attain as hereinafter set forth, reference being had to the accompanying drawings, in which,

Figure 1 is an elevation of a storage battery grid embodying our invention; and 30 Fig. 2 is a transverse section on the line 2—2, Fig. 1.

In accordance with our invention the alloy from which grids are to be made is melted in the ordinary manner and is cast in molds 35 evenly heated by suitable means, as for instance by electric heating units, so that the surfaces engaged by the metal of the casting are maintained at the same temperature in both parts of the mold and all parts of the 40 grid casting are cooled at the same rate during solidification. The mold temperature in addition to being uniform, is maintained at a point which will prevent such chilling of the metal as would render uncertain its 45 reaching and filling all parts of the mold, but is no higher at any point than is sufficient to attain this end. In other words, the temperature is below the melting point of the alloy, but is high enough to insure 50 the free flow in the mold of the molten alloy. Moreover we have found that the better flowing of the metal, due to the uniform mold heat, makes it possible to reduce not

only the mold temperature but the pouring 55 temperature of the metal, so that the finished product is free of blow holes, pores, or other minute as well as large cavities and is of increased density and uniform texture throughout its structure. 60

For insuring the above noted conditions we preferably employ a machine such as that described and claimed in the application for U. S. Patent of Messrs. Pearson and Holland #240,789, filed June 19, 1908 65 wherein the parts of the mold engaged by the casting are uniformly heated by electric heating units which permit the temperature to be regulated and maintained with the utmost accuracy and certainty. 70

We have found that battery plates having grids as above described have greater strength and will not buckle, warp or disintegrate under ordinary hard conditions of use since they are attacked to but a slight 75 extent and what small amount of electrochemical action does occur is uniformly distributed over the external surface of the grid metal and the electrolyte cannot penetrate as heretofore, into the interior structure of the metal through cavities or pores. 80

As this application contains matter in common with the application filed by us June 19, 1918, Serial Number 240,789, it is to be treated as a continuation of such 85 earlier application in so far as the common subject matter is concerned.

We claim:

1. A battery plate grid consisting of a lead alloy casting formed under temperature conditions such that its structure is substantially non-porous and homogeneous. 90

2. A battery grid consisting of a casting having all parts of its two faces formed of metal cooled at the same rate during solidification and substantially non-porous. 95

3. A battery grid consisting of a casting formed of lead alloy cast at a relatively low temperature just sufficient to permit it to fill all parts of an evenly heated mold. 100

4. The method of making a battery grid which consists in melting a lead alloy; and casting said alloy at a relatively low temperature in the form of a grid in an evenly heated, relatively cool mold. 105

5. The method of making a battery grid which consists in melting a lead alloy; cast

ing said alloy in the form of a grid; and cooling the grid with the surfaces of all parts thereof subjected to a uniform and controlled temperature above that of the atmosphere.

6. The method of making battery grids which consists in heating to and maintaining at the same temperature the two parts of a grid mold to be engaged by the molten metal; casting molten metal in said mold

while it is so heated; allowing the metal to solidify; and removing the cast grid.

7. A battery plate grid consisting of a lead alloy casting formed at a relatively low temperature such that its structure is substantially non-porous. 15

In witness whereof we affix our signatures.

LAWRENCE J. PEARSON.  
WALTER E. HOLLAND.